

## UNITED STATES PATENT OFFICE

HAROLD R. RAFTON, OF LAWRENCE, MASSACHUSETTS, ASSIGNEE TO RAFFOLD PROCESS CORPORATION, A CORPORATION OF MASSACHUSETTS

METHOD OF PRODUCING PAPER FILLED WITH ALKALINE FILLER

No Drawing. Application filed November 24, 1928, Serial No. 321,754. Renewed August 15, 1930.

This invention relates to the manufacture of paper and more particularly to a method of producing paper filled with alkaline filler.

The principal object of my invention is to provide a method for making either unsized or sized paper filler with alkaline filler wherein both alkaline filler and alum are added to a fibrous mix at such a point in the papermaking process that the time and intimacy of contact of the alkaline filler and alum in the mix are materially limited.

An important object of my invention is to provide a method for the reduction, elimination, prevention, or alteration of foam in the manufacture of substantially unsized paper filled with alkaline filler.

A further object of my invention is to improve paper machine operation in such manufacture, particularly as regards the dandy roll.

A further object is to avoid the deterioration by alkaline filler of the effect of alum in a paper mix.

A further object is to avoid the deterioration of a precipitate of size and alum by alkaline filler.

A further object is to avoid the deterioration of the precipitate formed by a soluble material such as sodium silicate and a precipitant such as alum in a paper filled with alkaline filler.

A further object is to provide a method of making paper filled with alkaline filler wherein alkaline filler and alum in conjunction with a soluble material such as size and/or other soluble material are added at such a point in the papermaking process that the time and intimacy of contact of the alkaline filler in the paper mix with the precipitates formed from these materials and alum are materially limited.

Another object is to provide a process wherein alkaline filler is employed, in which the "broke" may be fed to the beater.

Another object is to provide a process in

which the recovered stock from the white water may be re-utilized either in the beater or in one of the stuff chests.

Another object is to provide a cyclic process in which alkaline filler is used at the wet end of the paper machine in conjunction with alum, in which the "broke" from the machine is re-utilized in the beater and in which the constituents recovered from the white water are re-introduced at a point prior to that where the fibrous mix is diluted preparatory to delivery to the web-forming device of the paper machine.

Other objects and advantages of my invention will become apparent during the course of the following description.

In my copending applications Serial No. 304,167, filed September 5, 1928, and Serial No. 321,753, filed November 24, 1928, I have disclosed and claimed methods whereby sized and substantially unsized paper filled with alkaline filler may be made by adding alkaline filler at the wet end of the paper machine. Moreover in my copending applications Serial Nos. 304,168, 304,170, 304,171, 304,172, 304,173, 304,174, 304,176 and 304,177, all filed September 5, 1928, and in my copending applications Serial Nos. 319,719, and 319,720, both filed November 15, 1928, I have described and claimed various methods wherein alum is added at the wet end of the paper machine by which foaming may be prevented on the paper machine, by which better operation of the paper machine may be insured, by which sized papers may be made, by which material originally soluble may be incorporated into paper, all in the case of paper filled with alkaline filler.

In the applications mentioned above I have disclosed that certain effects produced by the addition in the beater of alum, or of alum and size, or of alum and soluble material such as sodium silicate, are deteriorated even up to the point of destruction by the presence of alkaline filler. As indicated, I have employed

two general methods which serve either to restore these effects which have been deteriorated or destroyed, or to prevent these effects from being destroyed, namely, the addition of alum at the wet end of the paper machine to a paper mix which already contains alkaline filler or the addition of alkaline filler at the wet end of the paper machine to a paper mix to which alum has already been added, and in which the effect desired to be produced already exists.

Cross references have been made in several of the applications to the possibility of the joint use of both of these methods under certain circumstances but claim has not been made thereto. In the present application claim is made to the joint use of these two methods both for sized and substantially unsized paper, and further disclosure as to advantages which inhere in a combination of these two methods is made.

My process consists substantially in adding originally all the fibrous constituents in the beater or similar machine, and then adding subsequently to these fibrous constituents the alkaline filler (not including alkaline filler admixed with fibrous constituents) and alum, together with size, if desired, and/or soluble material such as sodium silicate, at a point in the process where there will be a minimum of time and intimacy of contact of the constituents of the mix, that is at or subsequent to the point at which the relatively concentrated mix is diluted preparatory to delivery to the web-forming device of the paper machine, or in other words at the wet end of the paper machine.

The chief advantage of the employment of this method is the fact that "broke" containing alkaline filler may thereby be used directly in the beater. Furthermore the material recovered from the white water which of course contains alkaline filler may thereby be delivered directly into the beater or at any other point where the stock is still in concentrated condition, such for instance as in any of the stuff chests. This procedure permits the utilization of the equipment commonly used for white water recovery with the normally employed piping connections, instead of the changed piping required by the processes set forth in my copending applications Serial Nos. 304,167 filed September 5, 1928, and 321,753, filed November 24, 1928. Where the recovery system is of the filter or decker type, the "sweetener" stock may be taken exactly as is customary from one of the stuff chests and this stock together with the recovered material from the white water may be returned thereto or elsewhere into the concentrated stock system as desired.

Moreover the capacity of the beater for fibrous material is not reduced by the presence therein of alkaline filler. Furthermore the beating action is not retarded by the pres-

ence in the beater of material, i. e. filler, which mechanically covers the fibre and prevents full action thereon by the beater.

A further advantage is the tendency toward economy in alum as the alum and alkaline filler do not have an opportunity to react substantially within the brief time or under the conditions of dilution under which these two materials meet. Of course that portion, if any, of the alum accompanying the alkaline filler in the white water and returned through the recovery cycle will be acted upon.

My process is applicable as follows in the manufacture of paper filled with alkaline filler: firstly, for making a substantially unsized paper substantially free from foam marks; secondly, for producing a stock for paper which runs on the paper machine substantially free from dandy trouble; thirdly, for the manufacture of sized paper sized by any of the ordinary sizing materials, or by any of the special sizing agents set forth in my various copending applications mentioned above; fourthly, for preserving in stock and in the paper made therefrom the substantially undeteriorated effect imparted by a soluble material such as sodium silicate precipitated by a precipitant such as alum.

In the preferred practice of my invention I add in the beater fibrous material which may conveniently include the fibrous material which comes under the definition of alkaline filler hereinafter set forth in this specification. Other material such as coloring matter may also be added at this point if desired. After the usual subsequent treatment in the beater, the mix is preferably passed through the beater chest, Jordan, and machine chest in the customary manner. This exact procedure is not necessary and may be modified in accordance with the type of paper being made; moreover this placement of chests in respect to mechanical treating apparatus is subject to rearrangement as will be apparent to one skilled in the art. Where the machine is equipped with a decker or filter type of white water save-all, the "sweetener" stock may be drawn from one of the chests, and the stock, recovered from the white water combined with this "sweetener" stock, may be returned to the chest as is customary.

The relatively concentrated fibrous mix is now ready for dilution and is preferably at this point mixed with the alkaline filler, preferably in aqueous suspension. Of course white water, e. g. tray water, and other water is added as needed at this point. If, now, it is desired to use only alum as the additional material to be added to the mix, such as would be the case for example in the manufacture of substantially unsized paper where alum would be used for the purpose of preventing foam or improving machine operation or for any other use, the alum should now be added

to the dilute mix which contains the alkaline filler preferably thoroughly mixed therewith. If on the other hand it is desired to incorporate soluble material such as sodium silicate into the paper, or sizing material such as rosin size, or material such as an emulsion, e. g. a paraffin emulsion (together with an agent which mutually with a precipitating agent later to be added serves to concentrate the dispersed phase of said emulsion on the fibrous material), one or more of these materials may then be added to the diluted mix containing the alkaline filler, and when sufficient time has been given for them to be thoroughly mixed, the precipitating agent such as alum may then be added. Of course the alum may be added prior to these materials, and likewise of course the alkaline filler need not be added first, but the above is a suitable method for carrying out my invention. Moreover any two or more of the materials, preferably those which do not mutually react with one another, may be pre-mixed originally, such for example as the alkaline filler and rosin size solution, so as to necessitate a lesser number of materials to be mixed directly with the fibrous material at the wet end of the paper machine. Special mixing devices may be provided for incorporating the various materials with the fibrous mix, but usually the alkaline filler, preferably in aqueous suspension, is added at the point of dilution, and the other materials may be satisfactorily added successively, as the ordinary turbulence of the diluted mix, in the riffler for example, is sufficient to effect proper mixing. The ordinary time existing in machine operation between the point of dilution of the stock and its delivery to the web-forming device is usually amply sufficient to effect complete mixing. Of course the size and/or other soluble material such as sodium silicate may be previously added with the fibrous mix while the mix is in a relatively concentrated condition, but the important point is to add both the alkaline filler and the alum at the wet end of the paper machine. It is also possible of course to add the previously precipitated sizing and/or aluminum silicate at the wet end of the paper machine as set forth in my copending application Serial No. 304,175 filed September 5, 1928, and Serial No. 319,721, filed November 15, 1928, but I prefer to add the unprecipitated constituents separately.

55 The stock is now fed on to the web-forming device of the paper machine and the white water flowing therefrom may be returned cyclicly to the process. Part of this may be used as such in diluting the stock in the mixing box of the paper machine. Part, if desired, may be treated by sedimentation, filtration, deckering, or the like, recovering the matter in suspension therein for return to beater or chest, and returning as much of the clarified water as it may be feasible to

employ for re-use on the machine or in the rest of the papermaking operation.

An illustrative furnish suitable for the practice of my invention is as follows:

| <i>Materials added in the beater</i>                                                                            | <i>Pounds</i> |
|-----------------------------------------------------------------------------------------------------------------|---------------|
| Fibrous material (air dry basis), e. g. equal parts of sulphite pulp, soda pulp, and old paper stock            | 1550          |
| Broke (air dry basis), such as from the operation of the same machine or other broke containing alkaline filler | 75            |
| Alum                                                                                                            | 150           |
| <i>Materials to be added proportionately and continuously on dilution</i>                                       | <i>Pounds</i> |
| Alkaline filler (bone dry basis), e. g. calcium carbonate magnesium hydroxide                                   | 300           |
| Alum                                                                                                            | 35            |
|                                                                                                                 | 85            |

Another illustrative furnish is:

| <i>Materials added in the beater</i>                                                                            | <i>Pounds</i> |
|-----------------------------------------------------------------------------------------------------------------|---------------|
| Fibrous material (air dry basis), e. g. equal parts of sulphite pulp, soda pulp, and old paper stock            | 1550          |
| Broke (air dry basis), such as from the operation of the same machine or other broke containing alkaline filler | 150           |
| Alum                                                                                                            | 95            |
| <i>Materials added proportionately and continuously on dilution</i>                                             | <i>Pounds</i> |
| Alkaline filler (bone dry basis), e. g. calcium carbonate magnesium hydroxide                                   | 300           |
| Size, e. g. rosin size                                                                                          | 6             |
| Alum                                                                                                            | 40            |

Another illustrative furnish is:

| <i>Materials added in the beater</i>                                                                       | <i>Pounds</i> |
|------------------------------------------------------------------------------------------------------------|---------------|
| Fibrous material (air dry basis), e. g. equal parts of sulphite pulp, soda pulp, and old paper stock       | 1550          |
| Broke (air dry basis), as from the operation of the same machine or other broke containing alkaline filler | 150           |
| Alum                                                                                                       | 110           |
| <i>Materials added proportionately and continuously on dilution</i>                                        | <i>Pounds</i> |
| Alkaline filler (bone dry basis), e. g. calcium carbonate magnesium hydroxide                              | 300           |
| Inorganic alkali metal salt, e. g. 60° Be. sodium silicate                                                 | 40            |
| Precipitant, e. g. alum                                                                                    | 50            |
|                                                                                                            | 120           |

Another illustrative furnish is:

| <i>Materials added in the beater</i>                                                                       | <i>Pounds</i> |
|------------------------------------------------------------------------------------------------------------|---------------|
| Fibrous material (air dry basis), e. g. equal parts of sulphite pulp and soda pulp                         | 1550          |
| Broke (air dry basis), as from the operation of the same machine or other broke containing alkaline filler | 150           |

*Materials added proportionately and continuously on dilution*

|                                                                               | Pounds |
|-------------------------------------------------------------------------------|--------|
| Alkaline filler (bone dry basis), e. g. calcium carbonate magnesium hydroxide | 300    |
| Size, e. g. rosin size                                                        | 60     |
| Alum                                                                          | 85     |

It is to be understood that the above furnishes are illustrative only and not limiting, as I have found that my invention may be practiced with a wide variety of ingredients in the furnish, with widely varying proportions of the several ingredients to one another, for making a wide variety of grades of paper.

As will be apparent from the previous detailed discussion, it is very desirable to be able to utilize in a paper mix both a water soluble acidic constituent, alum, and a substantially water insoluble alkaline constituent, alkaline filler. These two materials, however, under conditions obtaining in the ordinary method of paper manufacture react chemically upon one another so that the effect of the alum is rapidly destroyed. The primary object of this invention is to so adjust conditions as to substantially prevent these two constituents from reacting chemically, and thus to preserve the desired effect of the alum in the paper-making mix. This result is attained as indicated above by adjusting conditions so that these two constituents are brought together in the paper mix under circumstances which tend to prevent their chemical reaction, that is, under conditions favoring the minimizing of the time and intimacy of contact of the constituents of the mix, or specifically, at the wet end of the paper machine. It is thus obvious that conditions are adjusted to prevent rather than to obtain a chemical reaction between the alum and the alkaline filler.

A chemical reaction between acidic material and alkaline material which is to result in a final state which is substantially in the vicinity of neutrality requires of course the employment of substantially chemically equivalent proportions of the two materials. Thus if it were desired to effect such a reaction between alum and alkaline filler, substantially chemical equivalents of each would have to be employed. A stoichiometrical calculation shows that if for example calcium carbonate were to be the alkaline filler used, 1 part thereof would be chemically equivalent to 2.2 parts of commercial alum. If calcium carbonate magnesium hydroxide (of equimolecular proportions) were to be the alkaline filler used, 1 part thereof would be chemically equivalent to 2.9 parts of alum.

In the present invention, however, no such chemically equivalent proportions of alkaline filler and alum are used, but rather the amount of alkaline filler used is far in excess

of the chemical equivalent of the alum used. This is made clear by reference to the first illustrative example of furnishes given above, in which the alkaline filler, in that case calcium carbonate magnesium hydroxide, has a ratio of filler to alum of 25 to 2.9. Thus it is apparent that in that case there is used 25 times the amount of alkaline filler which would be the chemical equivalent of the alum, that is, 25 times the amount of alkaline filler necessary to react completely with the alum were conditions provided favorable for the consummation of reaction between the two. In the other illustrative examples the ratio of filler to alum is somewhat lower and runs in the extreme case (fourth example) as low as 10.2 of alkaline filler to 2.9 of alum, that is, the alkaline filler is 10.2 times the chemical equivalent of the alum. This latter ratio, however, cannot be considered so representative of the ratio of the filler to alum employed in my invention as the ratio in the first example, because in the fourth illustrative furnish referred to there is present considerable amount of soluble alkaline material (size) which immediately removes a large part of the alum from the solution as an alum-size precipitate. Thus the actual "free" alum present, that is, the alum in excess of that needed to precipitate soluble constituents and which is actually the alum available for possible reaction with the alkaline filler, is considerably less than the total alum originally employed. Therefore the proportion of alkaline filler to free alum is actually much higher than 10.2 times the chemical equivalent of the alum as calculated above, and much nearer the 25 times given in the first example.

It is apparent therefore that I use an amount of alkaline filler far in excess of the chemical equivalent of the alum employed. Thus even were conditions such that the alkaline filler were acted upon by the alum, as is substantially not the case, under such conditions the unacted upon residual alkaline filler would only be slightly less in amount than that originally added, and thus substantially the same amount as added, (less, of course, the losses through the machine wire into the white water), would find its way into the paper. While I have not limited my invention to the addition of any definite amount of alkaline filler in relation to the total furnish, the examples of illustrative furnishes indicate that the proportion of alkaline filler normally present constitutes a substantial percentage of the total furnish, and thus the paper produced by my process will contain a substantial percentage of alkaline filler and will be what is known in the art as "paper filled with alkaline filler".

On the other hand if instead of using alkaline filler as is my practice in an amount greatly in excess of the alum used, alkaline

filler were employed only in an amount chemically equivalent to the alum used, it can be readily seen from the following computation that such an amount of alkaline filler would 5 not produce a paper which would be considered as a "paper filled with alkaline filler".

In order to compute the amount of alkaline filler that would be chemically equivalent in amount to the alum, it is only necessary to 10 know how much alum is ordinarily used. From the examples of illustrative furnishes above, it is apparent that whereas I have not limited my invention to the addition of any definite amount of alum in relation to 15 the total furnish, the proportion of alum used on the total furnish normally runs in the vicinity of several per cent. more or less. For example if I used 3% of free alum on the total furnish, which is somewhat more 20 than the average amount used in the illustrative furnishes, the amount of alkaline filler chemically equivalent thereto would be, in the case of calcium carbonate, about 1.4%, and in the case of calcium carbonate magnesium hydroxide about 1.1% on the total furnish. The resulting paper would, of course, 25 contain smaller percentages of filler owing to losses of filler through the machine wire into the white waters. Such amounts of filler, 30 therefore, or even amounts in some excess thereof, (such as would be present if the alkaline filler were used in amounts chemically equivalent to quantities of alum somewhat larger than the above assumed 3%), would 35 be wholly inadequate to impart any substantial degree of filling to the paper made with such furnish. Indeed, in such case analytical procedures of fairly exact degree of refinement would have to be employed to detect 40 the presence of such minute quantity of the alkaline filler as might find its way into the paper to distinguish it with certainty for instance from the small amounts of inorganic constituents naturally occurring in the fibres, 45 such as sulphite or soda fibers. On the other hand, the filler in paper ordinarily known as "filled" paper, such as that to which my invention is directed, is present in so much larger amount that the normal 50 inorganic constituents of the fibre are negligible in proportion thereto, and ordinary ashing of the paper by ignition gives a result indicating the filler content sufficiently accurately for practical paper mill purposes.

55 It is thus clearly evident that I add alkaline filler and alum at the wet end of the paper machine to prevent chemical reaction between the two and therefore my invention is completely differentiated from any paper-making procedure wherein an alkaline filler and alum in substantially chemically equivalent proportions are added to a papermaking mix for chemically reacting purposes. Moreover it is to be noted that where the procedure of adding substantially chemically

equivalent proportions of acid and alkali to a paper mix at the dilute stage has hitherto been employed, this chemical equivalence has according to the prior knowledge of the art been a necessary and limiting feature of such 70 procedure. Were more acid than alkali added, the desired minimizing of the acidity would have been defeated, and on the contrary were alkali substantially in excess of the chemical equivalent of the acid added, 75 the mix would have been alkalinized and the sizing would have been substantially deteriorated if not destroyed. The prior practice made no distinction between soluble and insoluble alkali. When substantially insoluble alkali

80 was used as a substitute for the soluble alkali it was subject to the same limitations as to quantity employed, and according to all known prior art the addition of an amount of insoluble alkali, e. g. alkaline filler, substantially in excess of that chemically equivalent to the acid added would have resulted in alkalinizing the mix to such an extent as to 85 substantially deteriorate if not destroy the sizing, and thus have defeated the purpose 90 for which it was added. It was not until the discovery herein disclosed, namely, that alkaline filler if added at the wet end of the paper machine would not substantially af-

fect the desirable acidic qualities in a paper 95 mix, that it was realized that an amount of alkaline filler greatly in excess of the chemical equivalent of the acidic constituent could be added at that point without thereby alkalinizing the mix. Hence the present in- 100

vention distinctly differentiates from any prior chemically reacting, i. e. neutralizing practice, as all such prior practice involving addition of both acid and alkali at the dilute stage was necessarily confined by the then 105 existing knowledge to the addition of substantially chemically equivalent proportions. It is also clear that my invention is directed to the manufacture of paper filled in substantial degree with alkaline filler, and it is thus 110

completely differentiated from any paper-making procedure in which alkaline filler and alum are added in chemically equivalent proportions, as in the latter case a commercially wholly inconsequential amount of al- 115

kaline filler, if indeed any quantity at all detectable by ordinary analytical procedure, is incorporated into the paper, and such paper cannot be considered in the ordinary paper-making interpretation of the words as "paper 120 filled with alkaline filler".

Instead of alum as a precipitant for the rosin size, I may use other salts of aluminum, or sodium bisulphate ( $\text{NaHSO}_4$ ) or the like; but from the standpoints of efficiency and 125 cost I prefer alum. In the case of the use of alum as a precipitant for sodium silicate, I may also substitute in addition to the above, ammonium salts such as the chloride or the sulphate.

Thus it will be apparent that certain of the equivalents of alum which I may use in the practice of my invention, e. g. other salts of aluminum and sodium bisulphate, may be classed with equal correctness either as "metallic salts" or as "acidic material".

Instead of sodium silicate, I may use sodium stannate or any of the other inorganic alkali metal salts with a pH value greater than 7.0, which are precipitable by material which depresses their hydroxyl ion concentration.

Instead of rosin size, which may be referred to as sodium resinate, and which may therefore be termed an alkali metal salt, any other size is suitable which is used in conjunction with a size precipitant as alum. One example of such a size is a soap, such as an oleate. Another is a wholly or partially saponified wax, such as beeswax. Or I may use special sizing agents e. g. those involving the use of paraffin emulsions as disclosed in several of my copending applications referred to above.

Where I use the expression "alkali metal", I mean to include the hypothetical alkali metal ammonium ( $\text{NH}_4$ ).

By the term "alkaline filler" I mean substantially water insoluble filler which when agitated in contact with freshly boiled distilled water, say for an hour, will impart a pH value to such water greater than 7.0, that is, which will be on the alkaline side of the neutral point. Among fillers included in this group may be mentioned calcium carbonate, of which lime mud from the causticizing process is one form; calcium carbonate magnesium basic carbonate employed in the paper disclosed in my U. S. Patent No. 1,595,416, issued August 10, 1926; calcium carbonate magnesium hydroxide disclosed in my U. S. Patent No. 1,415,391, issued May 9, 1922; and other substantially water insoluble normal or basic carbonates of alkaline earth metals (which expression is herein intended to include magnesium), or compounds, double salts, or physically associated mixtures of these with one or more other acid soluble materials of a substantially water insoluble nature.

By the term "alkaline filler" I also intend to include fibrous material and/or other material such as paper coating constituents or the like containing one or more compounds of the character referred to, such as "old papers" or similar papers, "broke", or the like.

When I use the word "paper" herein, I use it in the broad sense to include products of manufacture of all types and of all weights and thicknesses, which contain as an essential constituent a considerable amount of prepared fibre and which are capable of being produced on a Fourdrinier, cylinder, or other forming, felting, shaping or molding machine.

By the term "wet end of the paper machine" I intend to include those instrumentalities employed in paper manufacture by which and/or in which a relatively concentrated paper mix is diluted, and treated, conveyed or fed up to the point of web-formation, such as the mixing box, regulating and proportioning devices, rifflers, troughs, screens, head boxes, inlets, and the like, including also instrumentalities used in the white water cycle.

While I have described in detail the preferred embodiment of my invention, it is to be understood that the details of procedure, the proportions of ingredients, and the arrangement of steps may be widely varied without departing from the spirit of my invention or the scope of the subjoined claims.

I claim:

1. The method of manufacturing paper filled with alkaline filler comprising adding alkaline filler in an amount sufficient to impart a substantial degree of filling to the resulting paper, and an aluminum salt to fibrous material under conditions favoring the minimizing of time of contact, and thereafter making paper therefrom.

2. The method of manufacturing paper filled with alkaline filler comprising adding alkaline filler in an amount sufficient to impart a substantial degree of filling to the resulting paper, and an aluminum salt to fibrous material under conditions favoring the minimizing of intimacy and time of contact, and thereafter making paper therefrom.

3. The method of manufacturing paper filled with alkaline filler comprising adding alkaline filler in an amount sufficient to impart a substantial degree of filling to the resulting paper, and an aluminum salt to fibrous material at the wet end of the paper machine, and thereafter making paper therefrom.

4. The method of manufacturing paper filled with alkaline filler comprising adding alkaline filler in an amount sufficient to impart a substantial degree of filling to the resulting paper, and alum to fibrous material at the wet end of the paper machine, and thereafter making paper therefrom.

5. The method of manufacturing paper filled with alkaline filler comprising adding alkaline filler, in an amount sufficient to impart a substantial degree of filling to the resulting paper, soluble material, and an aluminum salt to fibrous material at the wet end of the paper machine, and thereafter making paper therefrom.

6. The method of manufacturing paper filled with alkaline filler comprising adding alkaline filler, in an amount sufficient to impart a substantial degree of filling to the resulting paper, soluble material comprising alkali metal salt, and an aluminum salt to fibrous material at the wet end of the paper

machine, and thereafter making paper therefrom.

7. The method of manufacturing paper filled with alkaline filler comprising adding 5 alkaline filler, in an amount sufficient to impart a substantial degree of filling to the resulting paper, soluble material comprising size, and an aluminum salt to fibrous material 10 at the wet end of the paper machine, and thereafter making paper therefrom.

15 8. The method of manufacturing paper filled with alkaline filler comprising adding alkaline filler, in an amount sufficient to impart a substantial degree of filling to the resulting paper, soluble material, and alum to fibrous material at the wet end of the paper machine, and thereafter making paper therefrom.

9. The method of manufacturing paper  
20 filled with alkaline filler comprising adding  
alkaline filler, in an amount sufficient to im-  
part a substantial degree of filling to the re-  
sulting paper, soluble material comprising  
rosin size, and an aluminum salt to fibrous  
25 material at the wet end of the paper machine,  
and thereafter making paper therefrom.

10. The method of manufacturing paper filled with alkaline filler comprising adding alkaline filler, in an amount sufficient to impart a substantial degree of filling to the resulting paper, soluble material comprising rosin size and an inorganic alkali metal salt with a pH value greater than 7.0, which is precipitable by material which depresses its hydroxyl ion concentration, and an aluminum salt to fibrous material at the wet end of the paper machine, and thereafter making paper therefrom.

11. The method of manufacturing paper  
40 filled with alkaline filler comprising adding  
alkaline filler, in an amount sufficient to im-  
part a substantial degree of filling to the re-  
sulting paper, soluble material comprising  
rosin size and sodium silicate, and an alumini-  
45 um salt to fibrous material at the wet end  
of the paper machine, and thereafter making  
paper therefrom.

12. The method of manufacturing paper filled with alkaline filler comprising adding 50 alkaline filler, in an amount sufficient to impart a substantial degree of filling to the resulting paper, soluble material comprising rosin size and sodium silicate, and alum to fibrous material at the wet end of the paper machine, and thereafter making paper therefrom.

13. The method of manufacturing paper filled with alkaline filler comprising adding alkaline filler consisting of alkaline earth metal compound, in an amount sufficient to impart a substantial degree of filling to the resulting paper, and an aluminum salt to fibrous material at the wet end of the paper machine, and thereafter making paper therefrom.

14. The method of manufacturing paper filled with alkaline filler comprising adding alkaline filler consisting of calcium carbonate, in an amount sufficient to impart a substantial degree of filling to the resulting paper, and an aluminum salt to fibrous material at the wet end of the paper machine, and thereafter making paper therefrom. 70

15. The method of manufacturing paper  
filled with alkaline filler comprising adding  
alkaline filler consisting of calcium carbonate  
and magnesium compound, in an amount suf-  
ficient to impart a substantial degree of filling  
to the resulting paper, and an aluminum salt  
to fibrous material at the wet end of the paper  
machine, and thereafter making paper there-  
from. 75  
80

16. The method of manufacturing paper filled with alkaline filler comprising adding alkaline filler consisting of calcium carbonate magnesium hydroxide, in an amount sufficient to impart a substantial degree of filling to the resulting paper, and an aluminum salt to fibrous material at the wet end of the paper machine, and thereafter making paper therefrom. 90

17. The method of manufacturing paper filled with alkaline filler comprising adding alkaline filler consisting of calcium carbonate magnesium hydroxide, in an amount sufficient to impart a substantial degree of filling to the resulting paper, soluble material, and an aluminum salt to fibrous material at the wet end of the paper machine, and thereafter making paper therefrom.

18. The method of manufacturing paper filled with alkaline filler comprising adding alkaline filler consisting of calcium carbonate magnesium hydroxide, in an amount sufficient to impart a substantial degree of filling to the resulting paper, soluble material comprising alkali metal salt, and an aluminum salt to fibrous material at the wet end of the paper machine, and thereafter making paper therefrom. 105 110

19. The method of manufacturing paper filled with alkaline filler comprising adding alkaline filler consisting of calcium carbonate and magnesium hydroxide, in an amount sufficient to impart a substantial degree of filling to the resulting paper, soluble material comprising size, and an aluminum salt to fibrous material at the wet end of the paper machine, and thereafter making paper therefrom. 115

20. The method of manufacturing paper filled with alkaline filler comprising adding alkaline filler consisting of calcium carbonate magnesium hydroxide, in an amount sufficient to impart a substantial degree of filling to the resulting paper, soluble material comprising rosin size, and an aluminum salt to fibrous material at the wet end of the paper machine, and thereafter making paper therefrom. 120 125

21. The method of manufacturing paper filled with alkaline filler comprising adding 130

alkaline filler consisting of calcium carbonate magnesium hydroxide, in an amount sufficient to impart a substantial degree of filling to the resulting paper, soluble material comprising size and sodium silicate, and an aluminum salt to fibrous material at the wet end of the paper machine, and thereafter making paper therefrom.

22. The method of manufacturing paper 10 filled with alkaline filler comprising adding alkaline filler consisting of calcium carbonate magnesium hydroxide, in an amount sufficient to impart a substantial degree of filling to the resulting paper, soluble material comprising size and sodium silicate, and alum to fibrous material at the wet end of the paper machine, and thereafter making paper therefrom.

23. The method of manufacturing paper 20 filled with alkaline filler, comprising adding alkaline filler, in an amount sufficient to impart a substantial degree of filling to the resulting paper, and an aluminum salt at the wet end of the paper machine to fibrous material comprising sulphite and soda pulps, and thereafter making paper therefrom.

24. The method of manufacturing paper 30 filled with alkaline filler, comprising adding alkaline filler, in an amount sufficient to impart a substantial degree of filling to the resulting paper, and an aluminum salt at the wet end of the paper machine to fibrous material comprising sulphite and soda pulps and old paper stock, and thereafter making paper therefrom.

35 25. The method of manufacturing paper 40 filled with alkaline filler comprising adding fibrous material in the beater, alkaline filler, in an amount sufficient to impart a substantial degree of filling to the resulting paper, and alum at the wet end of the paper machine, and thereafter making paper therefrom.

26. The cyclic procedure in a method of 45 manufacturing paper filled with alkaline filler comprising the addition at the wet end of the paper machine of alkaline filler, in an amount sufficient to impart a substantial degree of filling to the resulting paper, and alum, and the returning of the material recovered from the white water to the fibrous material while the same is in a relatively concentrated condition.

27. The cyclic procedure in a method for 55 the manufacture of paper filled with alkaline filler comprising the addition at the wet end of the paper machine of alkaline filler, in an amount sufficient to impart a substantial degree of filling to the resulting paper, and alum, the returning of the material recovered from the white water to the fibrous material 60 while the same is in a relatively concentrated condition, and the returning of the broke from said manufacture to the beater.

28. That step in a method of manufacturing paper filled with alkaline filler which 65 comprises adding alkaline filler, in an amount

sufficient to impart a substantial degree of filling to the resulting paper, and acidic material to fibrous material at the wet end of the paper machine.

29. That step in a method of manufacturing paper filled with alkaline filler which comprises adding alkaline filler, in an amount sufficient to impart a substantial degree of filling to the resulting paper, and metallic salt to fibrous material at the wet end of the paper machine.

30. That step in a method of manufacturing paper filled with alkaline filler which comprises adding alkaline filler, in an amount sufficient to impart a substantial degree of filling to the resulting paper, and aluminum compound to fibrous material at the wet end of the paper machine.

31. That step in a method of manufacturing substantially unsized paper filled with alkaline filler which comprises adding alkaline filler, in an amount sufficient to impart a substantial degree of filling to the resulting paper, and acidic material to fibrous material at the wet end of the paper machine.

32. That step in a method of manufacturing substantially unsized paper filled with alkaline filler which comprises adding alkaline filler, in an amount sufficient to impart a substantial degree of filling to the resulting paper, and metallic salt to fibrous material at the wet end of the paper machine.

33. That step in a method of manufacturing substantially unsized paper filled with alkaline filler which comprises adding alkaline filler, in an amount sufficient to impart a substantial degree of filling to the resulting paper, and aluminum compound to fibrous material at the wet end of the paper machine.

In testimony whereof I affix my signature.

HAROLD ROBERT RAFTON.